

1

3,374,171

**AQUEOUS LUBRICANT COMPOSITIONS CONTAINING AN ALKANOLAMINE, A SATURATED ORGANIC ACID AND A POLYOXY-ALKYLENE GLYCOL**

Robert H. Davis, Pitman, N.J., assignor to Mobil Oil Corporation, a corporation of New York  
No Drawing. Continuation-in-part of application Ser. No. 505,454, Oct. 28, 1965. This application Apr. 25, 1967, Ser. No. 633,416

10 Claims. (Cl. 252—34.7)

**ABSTRACT OF THE DISCLOSURE**

Lubricant compositions are provided containing a major proportion of water and minor amounts of a water-soluble alkanolamine, a saturated organic acid having from about 6 to about 9 carbon atoms per molecule and a polyoxyalkylene glycol. These compositions are particularly effective as cutting fluids in metal machining operations.

**CROSS REFERENCES TO RELATED APPLICATIONS**

Parent applications: Application Ser. No. 505,454, filed Oct. 28, 1965, now abandoned. Application Ser. No. 569,598, filed Aug. 2, 1966, and now abandoned.

**BACKGROUND OF THE INVENTION****1. Field of the invention**

This application, which is a continuation-in-part of my application Ser. No. 505,454, filed Oct. 28, 1965, now abandoned, and a continuation-in-part of my copending application Ser. No. 569,598, filed Aug. 2, 1966, and now abandoned, relates to lubricant compositions and, more particularly, to aqueous compositions adapted for use as lubricants and coolants in metal machining operations.

**2. Description of the prior art**

In machining operations of metals, such as cutting, grinding, turning, milling and the like, it is customary to flood the tool and the work with a coolant for the purpose of carrying off heat which is produced during the operation. It is also customary to employ these coolants in combination with various agents having lubricating and extreme-pressure properties for reducing friction between the tool and work piece, particularly in operations such as tapping and broaching. In this respect, it has, heretofore, been the practice to employ for such purpose aqueous compositions containing such lubricating agents as emulsified petroleum or non-petroleum additives. Such aqueous cutting fluids, in order to perform satisfactorily, should meet certain important requirements.

Among the requirements for a satisfactory cutting fluid are corrosion-inhibiting properties for ferrous and cuprous alloys, and also stability under the conditions of operation. While various cutting fluids may possess such characteristics, there are, however, further important requirements that should also be met. Among these requirements is the ability to avoid leaving deposits on the tool and the work following the machining operation which result from subsequent drying of the fluid and which are difficult to remove. Other important requirements include tolerance in hard water solutions so that the precipitation of lubricant components will not occur, avoidance of tacky residues which interfere with the operation of the machine and avoidance of excessive foam formation. Cutting fluids known prior to this invention have not, however, satisfactorily met all of the foregoing requirements.

2

**Summary of the invention**

It has now been found that a balanced formulation can be obtained in a lubricant composition which is effective as a cutting fluid having improved corrosion-resistant lubricating and cooling efficiency properties and which, in the course of machining operations, maintains its transparency in hard water solutions, avoids the formation of tacky water-insoluble residues, is free from excessive foam formation and is resistant to rancidity.

10 The foregoing improvements, as more fully hereinafter described, are, in general, realized with aqueous compositions comprising a balanced formulation and containing as essential components a major proportion of water and, in individual minor proportions, the combination of a saturated organic acid, either straight-chain or branched-chain having from about 6 to about 9 carbon atoms per molecule, a water-soluble alkanolamine and a water-soluble polyoxyalkylene glycol. In this respect, it is found that the alkanolamine component, in addition to functioning as a corrosion-inhibiting agent in which the aforementioned organic acids are soluble, also functions as a plasticizer in that, in the course of use, evaporation of water from the cutting fluid leaves a residue upon machinery parts which is desirably soft or semi-liquid. The function of the organic acid component in combination with the alkanolamine is primarily that of a corrosion inhibitor in that it forms the corresponding amine acid salt. The water-soluble polyoxyalkylene glycol in the novel composition functions as a load-support agent.

25 The water-soluble alkanolamine employed in the novel formulation may be of any molecular weight but should, preferably, be liquid at room temperature. The lower molecular weight compounds are generally preferred and, for this purpose, it has been found that such alkanolamines as mono-, di- or tri-ethanolamine are most effective. Other water-soluble alkanolamines may also be employed, and include such alkanolamines as iso-propanolamines, e.g., mono-, di- and tri-isopropanolamine, di-methyl-ethanolamine, diethyl-ethanolamine, aminoethyl-ethanolamine, N-acetyl ethanolamine, phenylethanolamine, phenyldiethanolamine and mixtures thereof.

30 The organic acid component, as previously indicated, comprises a saturated organic acid, either straight-chain or branched-chain having from about 6 to about 9 carbon atoms per molecule, or mixtures thereof. In this respect, it has been found that the relatively lower molecular weight acids having from about 1 to about 5 carbon atoms per molecule do not satisfactorily function as rust inhibitors and are also objectionable because of their strong odor. On the other hand, it is found that by employing relatively high molecular weight saturated organic acids, i.e., acids having more than about 9 carbon atoms per molecule, there results poor hard water stability, reduced corrosion inhibiting properties and high foaming tendencies. Of particular utility with respect to the aforementioned saturated intermediate molecular weight organic acids in the present improved formulation are hexanoic, heptanoic, caprylic and pelargonic acids.

35 In combination with the aforementioned water-soluble alkanolamines and saturated organic acids is the use of the water-soluble polyoxyalkylene glycols as load-support agents. Preferred compounds of this type include water-soluble oils obtained by copolymerizing mixtures of ethylene oxide and propylene oxide, e.g., oils prepared by copolymerizing a 50-50 mixture of ethylene oxide and propylene oxide; water-soluble heteric copolymeric alkylene glycols, ethers or esters thereof, wherein the different oxyalkylene units are substantially, randomly distributed throughout the entire polyoxyalkylene chain; water-soluble polyoxyalkylene compounds containing hydrophobic homopolyoxyalkylene

units; and polymeric agents, in general, which are block copolymers of cogeneric mixtures of conjugated polyoxyalkylene compounds containing at least one hydrophobic homopolyoxyalkylene unit, having a unit weight of at least about 800, and one or two other hydrophilic polymeric units which comprise from about 15 percent to about 90 percent of the total polymeric compound. The most desirable water-soluble polyoxyalkylene glycols for use in the formulations of the present invention comprise the polyether polyols produced by reacting ethylene oxide and propylene oxide having hydroxyl numbers from about 22 to about 38. If so desired, in order to impart increased anti-rust properties to the aqueous lubricant composition, an alkali metal nitrite may also be employed in the novel formulation. In this respect, it is found that more specific increased resistance to copper corrosion may also be obtained by the additional use of the sodium salt of mercapto-benzothiazole or benzotriazole.

The aforementioned novel formulations of water-soluble alkanolamine, saturated organic acid and water-soluble polyoxyalkylene glycol may also include a wide variety of germicidal agents for inhibiting bacterial growth. For this purpose, the germicidal agent may comprise, for example, a halogenated cresol, either completely or partially halogenated, and may include such representative compounds as completely or partially chlorinated, brominated, fluorinated or iodated cresols. Typical examples of this class of materials include: chloro-, dichloro-, trichloro-, and tetrachlorocresols; bromo-, dibromo-, tribromo, and tetrabromocresols, or any of the aforementioned compounds in which the chlorine or bromine atoms are substituted in whole or in part by fluorine or iodine. More specific compounds include: para-chloro-meta-cresol; para-bromo-meta-cresol; para-fluoro-meta-cresol; para-iodo-meta-cresol; 2,4-dichloro-meta-cresol; 2,4,5-trichloro - meta-cresol; 2,4,5,6-tetrachloro-meta-cresol; 2,4 - dibromo-meta-cresol; 2,4,5-tribromo-meta-cresol; 2,4,5,6 - tetrabromo-meta-cresol; or any of the aforementioned compounds in which the chlorine or bromine atoms are substituted in whole or in part by fluorine or iodine; or any corresponding ortho or para-cresols of the aforementioned compounds substituted for the corresponding meta-cresols.

Other germicidal agents that may be employed in the above-described novel formulations may include microbicidal gases, for example, in the form of aldehydes, such as formaldehyde, or aldehyde-releasing agents, such as formaldehyde-releasing agents, i.e., materials which break down in storage to form the aldehyde or aldehyde compounds as decomposition products. Thus, it is found that compounds of the type such as tris(hydroxymethyl)nitromethane are particularly effective in releasing formaldehyde and thereby providing germicidal protection over relatively long periods of time. Other microbicidal gases that may be employed for this purpose include ethylene oxide and beta propiolactone. Alcohols such as methyl alcohol, ethyl alcohol or higher alcohols may also be employed as germicidal agents. Other effective germicidal agents include halogens and halogen compounds, particularly iodine and chlorine and compounds of these halogens. Specific compounds of this type may include chloride of lime and iodophors. Furthermore, as germicidal agents, compounds of heavy metals may also be employed in the novel formulations. These may include such compounds as bichloride of mercury and organic mercurials such as Mercurochrome, Merthiolate, Metaphen, silver nitrate and copper sulfate. Germicidal agents comprising phenol and its derivatives may also be employed in the novel formulations, which include the aforementioned cresols and bis-phenols. Synthetic detergents may also be employed as germicidal agents, which are of the non-phenolic type. These may include, for example, ammonium halides, such as ammonium chloride, in which the hydrogen atoms have

been replaced by organic radicals; particularly effective are quaternary compounds in which the long-chain organic radical (alkyl group) contains from 12 to 16 carbon atoms. Other materials include quaternary compounds in which the organic group is an anion, e.g., sodium lauryl-sulfate, as well as those compounds which do not ionize.

The novel lubricant compositions of the present invention, as previously indicated, are formulated in accordance with certain balanced proportions expressed in weight percent. Thus, with water being present in a major proportion in each instance, the alkanolamine is employed in an amount from about 5 to about 40 percent, and preferably in an amount from about 20 to about 35 percent, 10 by weight. The organic acid component is employed in an amount from about 0.1 to about 9 percent, and preferably in an amount from about 1 to about 4 percent, by weight. The polyoxyalkylene glycol is employed in an amount from about 0.5 to about 20 percent, and 15 preferably in an amount from about 0.5 to about 5 percent, by weight. Where a germicidal agent is also to be incorporated in the novel formulation, these agents are employed in an amount from about 0.05 to about 5 percent, and 20 preferably in an amount from about 0.5 to about 3 percent, by weight. When the alkali metal nitrite is to be included in the formulation, it is generally employed in an amount from about 0.1 to about 10 percent, and 25 preferably in an amount from about 0.1 to about 5 percent, by weight. When the sodium salt of mercapto-benzothiazole is to be included in the formulation, it is generally present in an amount from about 0.1 to about 6 percent, and 30 preferably from about 0.1 to about 3 percent, by weight. If so desired, other additives for enhancing rust protection or for the purpose of raising the pH of the 35 system may be employed. Such additional additives may include boric acid or oxides of boron for enhancing rust protection, and are generally employed in an amount from about 0.1 to about 5 percent, and preferably from about 0.1 to about 3 percent, by weight. For raising the 40 pH of the system, such additional additives may be employed in the form of alkali metal hydroxides, including, more specifically, sodium, lithium or potassium hydroxide. When the latter are present, they are generally employed in an amount from about 0.1 to about 3 percent, and 45 preferably from about 0.1 to about 1.5 percent, by weight. Furthermore, if so desired, various water-soluble chelating agents may be employed to soften the water vehicle. These may include, for example, salts of ethylenediamine 50 tetraacetic acid, nitrilo-triacetic acid or diethylene triamine pentaacetic acid. When any of the aforementioned chelating agents are employed, they are generally present in an amount from about 0.1 to about 5 percent, by weight. In each instance, of course, it will be apparent that sufficient water is employed in order to balance the 55 formulation.

The novel lubricant compositions of the present invention are preferably prepared by a blending procedure which comprises reacting the alkanolamine and organic acid components with about 10 to about 20 parts of water, which is to be present in the finished formulation. 60 This blending procedure may be carried out at room temperature. However, heating to 120° F. with agitation is most satisfactory. The remaining quantity of water required to be present in the finished product is added, together with the polyoxyalkylene glycol, and any of the 65 aforementioned other desired components. It should be noted, however, that if an alkali metal nitrite is to be present in the finished product, such material is added last for the reason that addition of acids such as caprylic acid to a solution of sodium nitrite could result in decomposition of the nitrite, thus reducing or nullifying its 70 rust-inhibiting effects. If a germicidal agent is to be incorporated in the novel formulation, it is preferably 75 blended with the alkanolamine and organic acid.

## DESCRIPTION OF SPECIFIC EMBODIMENTS

The compounding of the novel compositions of the present invention may be illustrated by the preparation of lubricant and cutting fluids from the formulations in the following tables and examples and which also include comparative data and the observations noted when compositions are prepared which do not include all of the essential saturated organic acid, alkanolamine and polyoxy-alkylene glycol components of the present improved formulations. In this respect, as indicated above, among the outstanding properties of the improved lubricant compositions of the present invention are their rust-inhibiting properties, hard water stability and high machining efficiency. Accordingly, these improved compositions were subjected for the purpose of evaluation to the following corrosion, hard water stability and machining efficiency tests:

## Corrosion test

One to three grams of malleable iron turnings are placed in a glass container, washed with the test solution which is to be evaluated, drained and allowed to stand in an atmosphere of approximately 90 percent relative humidity and at a temperature of about 70° F. for a period of about 72 hours. After this period the sample is then checked for the appearance of rust. The samples are graded from 0 (no rust) to 3 (severe rusting) in accordance with the following standard chart. This test, and a more detailed general method for carrying it out is described in Patent No. 3,071,545, issued Jan. 1, 1963.

## Description:

|                                                                                                               | Rating |
|---------------------------------------------------------------------------------------------------------------|--------|
| No rusting, or less than 1% of the metal surface coated with yellow iron oxide                                | 0      |
| Light rusting, rusting confined to not more than six spots, each of which is 1 mm. or less in diameter        | 1      |
| Moderate rusting, rusting in excess of the above, but confined to less than 5% of the surface of the specimen | 2      |
| Severe rusting, rusting covering more than 5% of the surface of the specimen                                  | 3      |

5  
cant compositions of the present invention is evaluated with respect to a series of holes, drilled in a test bar made from hot-rolled steel, which are to be tapped. Prior to testing, samples of the novel formulations are diluted by employing 1 part, by weight, of the additive concentrate to 5 parts, by weight, of distilled water. The fluid is applied to the tap with a polyethylene squeeze-bottle. Four unknown samples are bracketed by two standards. The tapping efficiency is calculated by dividing the torque obtained with the unknown, into the average standard torque, and multiplying by 100. This test, and a more detailed general method for carrying it out is described in Patent No. 3,071,545, issued Jan. 1, 1963.

10  
15  
In the following Table I, samples containing triethanolamine, a polyether polyol, in the form of a copolymer, produced by reacting ethylene oxide and propylene oxide, and having a hydroxyl number from about 22 to about 38, and a saturated organic acid having from 4 to 9 carbon atoms per molecule, were subjected to the aforementioned corrosion test, in which the composition of the hard water employed was derived from that described in ASTM Test 1478-57T, paragraph 4a, which shows a preponderance of magnesium and sulfate ions. This water was modified in two ways, viz., the active ingredients were increased by 20  
25  
50 per cent, in order to increase total hardness from about 230 p.p.m. to about 345 p.p.m. and to increase the sulfate content to about 270 p.p.m. Sodium hydroxide was used to neutralize excess carbon dioxide employed for stabilization to attain a neutral pH.

30  
35  
As will be seen from Table I the samples containing triethanolamine, the ethylene oxide-propylene oxide copolymer, and either hexanoic, heptanoic, caprylic or pelargonic acids (Examples 3, 4, 5, and 6) effectively inhibited rusting of the malleable iron turnings, with a rating, in each instance, of 0. On the other hand, where the acid component comprised valeric or isobutyric acids, (Examples 1 and 2), severe rusting occurred with a rating of 3, clearly indicative of the fact that when the acid 40  
20  
component contains less than 6 carbon atoms per molecule, it is unsatisfactory for use in metal working operations.

TABLE I.—AQUEOUS SYSTEMS CONTAINING AN ALKANOLAMINE SALT OF SATURATED C<sub>4</sub>-C<sub>9</sub> ORGANIC ACID AND ETHYLENE OXIDE-PROPYLENE OXIDE COPOLYMER

| Ex. No. | Base Formula                     |                                  |                               |                                |                                 |                                |                                  |                            | Malleable Iron Rust-Test |
|---------|----------------------------------|----------------------------------|-------------------------------|--------------------------------|---------------------------------|--------------------------------|----------------------------------|----------------------------|--------------------------|
|         | Triethanolamine<br>(Percent Wt.) | Isobutyric Acid<br>(Percent Wt.) | Valeric Acid<br>(Percent Wt.) | Hexanoic Acid<br>(Percent Wt.) | Heptanoic Acid<br>(Percent Wt.) | Caprylic Acid<br>(Percent Wt.) | Pelargonic Acid<br>(Percent Wt.) | Copolymer<br>(Percent Wt.) |                          |
| 1       | 20                               | 3                                |                               |                                |                                 |                                |                                  | 7                          | 70                       |
| 2       | 20                               |                                  | 3                             |                                |                                 |                                |                                  | 7                          | 70                       |
| 3       | 20                               |                                  |                               | 3                              |                                 |                                |                                  | 7                          | 70                       |
| 4       | 20                               |                                  |                               |                                | 3                               |                                |                                  | 7                          | 70                       |
| 5       | 20                               |                                  |                               |                                |                                 | 3                              |                                  | 7                          | 70                       |
| 6       | 20                               |                                  |                               |                                |                                 |                                | 3                                | 7                          | 70                       |

## Hard water stability test

In this test, 1 part of the aqueous metal working fluid is mixed with 5 parts of the aforementioned ASTM 1478-57T, paragraph 4a, hard water of Table I, below, and stored in a 100 ml. graduated cylinder, for a period of 72 hours, at a temperature between about 70° F. and about 75° F. At the end of this period, there is recorded the volume of sediment formed as a result of interaction between the additives in the cutting fluid and the polyvalent ions present in the water.

## Machining efficiency test

The machining efficiency of the novel improved lubri-

65  
70  
In the following Table II, samples containing triethanolamine, a copolymer of ethylene oxide and propylene oxide, as recited in Table I, and a saturated organic acid having from 6 to 10 carbon atoms per molecule, were subjected to a hard water stability test, which was carried out in the following manner: One part of the specific aqueous metal working fluid was mixed with five parts of the ASTM hard water, as described in Table I, and stored in a 100 ml. graduate cylinder for a period of 72 hours and at a temperature from about 70° F. to about 75° F. At the end of this period, the volume of sediment formed as a result of interaction between the additives in the cutting fluid and polyvalent ions present in the water, were recorded.

As will be seen from Table II, the samples containing triethanolamine, the ethylene oxide-propylene oxide copolymer, and either hexanoic, heptanoic, caprylic or pelargonic acids (Examples 1, 2, 3, and 4), revealed no separation after 72 hours. On the other hand, where the acid component comprised capric acid (Example 5), a white insoluble soap (10% by volume) appeared at the top of the graduate. This outstanding difference, with reference to saturated organic acids having more than 9 carbon atoms per molecule, is indicative of the fact that the use of such higher organic acids can result in clogged filters, poor rust protection and reduced tool life in areas where hard water is encountered.

In order to illustrate the efficacy and criticality of employing a germicidal agent, such as a halogenated cresol, in the lubricating compositions of the present invention in combination with the aforementioned alkanolamine, organic acid and polyoxyalkylene glycol components, a series of comparative tests were conducted in which the aforementioned halogenated cresol, as represented by para-chloro-meta-cresol, and also other related germicidal agents, were evaluated for their effect in inhibiting bacterial growth in the otherwise identical lubricating composition.

The test employed for the aforementioned purpose is a biocide screening test employing a shaker method and, in

TABLE II.—AQUEOUS SYSTEMS CONTAINING AN ALKANOLAMINE SALT OF SATURATED C<sub>6</sub>–C<sub>10</sub> ORGANIC ACID AND ETHYLENE OXIDE-PROPYLENE OXIDE COPOLYMER

| Ex. No. | Base Formula                  |                             |                              |                             |                               |                           |                         | Hard Water Stability Test     |                                                                                |
|---------|-------------------------------|-----------------------------|------------------------------|-----------------------------|-------------------------------|---------------------------|-------------------------|-------------------------------|--------------------------------------------------------------------------------|
|         | Triethanolamine (Percent Wt.) | Hexanoic Acid (Percent Wt.) | Heptanoic Acid (Percent Wt.) | Caprylic Acid (Percent Wt.) | Pelargonic Acid (Percent Wt.) | Capric Acid (Percent Wt.) | Copolymer (Percent Wt.) | Distilled Water (Percent Wt.) | Percent Volume Separation<br>1 part base formula to 5 parts<br>ASTM Hard Water |
| 1-----  | 20                            | 3                           | -----                        | -----                       | -----                         | -----                     | 7                       | 70                            | No separation.                                                                 |
| 2-----  | 20                            | -----                       | 3                            | -----                       | -----                         | -----                     | 7                       | 70                            | Do.                                                                            |
| 3-----  | 20                            | -----                       | -----                        | 3                           | -----                         | -----                     | 7                       | 70                            | Do.                                                                            |
| 4-----  | 20                            | -----                       | -----                        | -----                       | 3                             | -----                     | 7                       | 70                            | Do.                                                                            |
| 5-----  | 20                            | -----                       | -----                        | -----                       | -----                         | 3                         | 7                       | 70                            | 10% white insoluble residue.                                                   |

In order to illustrate the importance of the aforementioned polyoxyalkylene glycol as an effective load-support agent in the novel aqueous lubricant compositions of the present invention, it will be seen from the following Table III, that neither the triethanolamine, nor the aforementioned ethylene oxide-propylene oxide copolymer, when used alone, or mixtures thereof (as in Examples 1, 2 and 3) are effective load-support agents, as indicated by the respective tapping efficiency, in each case, which is below 79 percent. Furthermore, as will be seen from Table III, the amine salts of the aforementioned C<sub>6</sub>–C<sub>9</sub> saturated organic acids, as represented by heptanoic, caprylic, and the branched-chain 2-ethyl hexoic acid, are more effective, but the tapping efficiency results are still below 89 percent. It will be noted, however, that a combination of the aforementioned ethylene oxide-propylene oxide copolymer and the aforementioned amine salts, produces tapping efficiency results which range from 93 to 96 percent (as in Examples 5, 7 and 9). This represents a significant increase in tapping efficiency over the aforementioned amine salts when used alone (as in Examples 4, 6 and 8). It will, therefore, be apparent that there is a synergistic extreme pressure effect between the aforementioned polyoxyalkylene glycol and the amine salts.

general, involves dilution of the cutting fluid to be evaluated with sterile nutrient broth (nutrient broth is used in place of distilled water in order to accelerate bacterial growth); inoculation from a standard bacterial culture; and incubation for a period of 48 hours at 30° C. Bacterial growth is considered proportional to the increase in turbidity of the sample.

More specifically, the aforementioned biocide screening test, which is used to determine bactericidal activity by visual observation of change in turbidity of a challenged solution, is carried out in the following manner. The nutrient broth is prepared having the following components, by weight:

|                       | Percent |
|-----------------------|---------|
| Peptone -----         | 0.5     |
| Beef extract -----    | 0.3     |
| Distilled water ----- | 99.2    |

In accordance with the above-indicated proportions, the peptone and beef extract are added to the water and the resulting mixture is sterilized (autoclaved at 270° F. for 30 minutes). The sterile broth is then removed from the autoclave and allowed to cool to ambient temperature.

The contents of one ampoule of freeze-dried bacteria

TABLE III.—AQUEOUS SYSTEMS CONTAINING AN ALKANOLAMINE, OR SATURATED ORGANIC ACID OR ETHYLENE OXIDE-PROPYLENE OXIDE COPOLYMERS, OR MIXTURES THEREOF

| Example No. | Base Formula                  |                              |                             |                                   |                         |                               | Tapping Efficiency, Percent 1-5 Dilution, Base Formula-Dist. Water |
|-------------|-------------------------------|------------------------------|-----------------------------|-----------------------------------|-------------------------|-------------------------------|--------------------------------------------------------------------|
|             | Triethanolamine (Percent Wt.) | Heptanoic Acid (Percent Wt.) | Caprylic Acid (Percent Wt.) | 2-Ethyl Hexoic Acid (Percent Wt.) | Copolymer (Percent Wt.) | Distilled Water (Percent Wt.) |                                                                    |
| 1-----      | 30                            | -----                        | -----                       | -----                             | -----                   | 70                            | 75.7                                                               |
| 2-----      | -----                         | -----                        | -----                       | 30                                | 70                      | 78.7                          |                                                                    |
| 3-----      | 20                            | -----                        | -----                       | -----                             | 10                      | 70                            | 75.5                                                               |
| 4-----      | 20                            | 10                           | -----                       | -----                             | -----                   | 70                            | 81.0                                                               |
| 5-----      | 20                            | 3                            | -----                       | -----                             | 7                       | 70                            | 95.5                                                               |
| 6-----      | 20                            | -----                        | 10                          | -----                             | -----                   | 70                            | 81.7                                                               |
| 7-----      | 20                            | -----                        | 3                           | -----                             | 7                       | 70                            | 96.0                                                               |
| 8-----      | 20                            | -----                        | -----                       | 10                                | -----                   | 70                            | 87.5                                                               |
| 9-----      | 20                            | -----                        | -----                       | 3                                 | 7                       | 70                            | 93.0                                                               |

From the foregoing, it will be apparent that the novel aqueous lubricant compositions of the present invention comprising an alkanolamine, a saturated organic acid having from about 6 to about 9 carbon atoms per molecule, and a polyoxyalkylene glycol, exhibit outstanding properties as evidenced from the above-described data, from a standpoint of corrosion-resistance, hard water stability and machining efficiency.

inoculum (primarily *staphylococcus albus*), which yields approximately 634 million bacteria per milliliter when the contents of the ampoule are added to 25 ml. of sterile nutrient broth and are incubated for 24 hours at 30° C., is added to 100 ml. of nutrient broth prepared in accordance with the above-described procedure in a 500 ml. Erlenmeyer flask. The flask and contents are placed in an incubator overnight at a temperature of 30° C. for growth.

At the end of this period, the flask is removed and 10 ml. of sterile glycerol are added and mixed for a period of one minute. Vials are prepared containing 2 ml. of this mixture (inoculum) and placed in a freezer until needed.

20 ml. of the nutrient broth, prepared as previously described, are added to a 50 ml. Erlenmeyer flask which is plugged with cotton and autoclaved for 30 minutes at 270° F. The flask is then removed from the autoclave and allowed to cool at ambient temperature. 0.5 ml. of the inoculum and 0.5 ml. of the sample under test are then added to the flask which is again plugged with sterile cotton and placed in an incubator shaker for 48 hours at 30° C. The presence of turbidity at the end of a test period indicates bacterial growth and, therefore, failure in the test.

Table IV, below, shows the data obtained in which a halogenated cresol as typical of the germicides of the present invention, and as represented by para-chloro-meta-cresol and other related germicidal agents, were evaluated for their bacterial growth-inhibiting effects.

2. The lubricant composition of claim 1 wherein said alkanolamine is present in an amount from about 20 to about 35 percent, by weight; said organic acid is present in an amount from about 1 to about 4 percent, by weight; and said polyoxyalkylene glycol is present in an amount from about 0.5 to about 5 percent, by weight.

3. The lubricant composition of claim 1 containing as an additional component a germicidal agent selected from the group consisting of halogenated cresols, aldehydes, formaldehyde and tris (hydroxymethyl)nitromethane in an amount from about 0.05 to about 5 percent, by weight.

4. A lubricant composition containing a major proportion of water; a water-soluble alkanolamine in an amount from about 5 to about 40 percent, by weight; a saturated organic acid having from about 6 to about 9 carbon atoms per molecule, selected from the group consisting of straight-chain organic acids and branched-chain organic acids, in an amount from about 0.1 to about 9 percent, by weight; a water-soluble polyoxyalkylene glycol in an amount from about 0.5 to about 20 percent, by weight;

TABLE IV.—BIOCIDE SCREENING TEST—SHAKER METHOD

| Ex. No. | Base Formula                   |                             |                                      |                                     |                                      |                      |                                             |                               | Bacterial growth rating 0.5 part base formula 20 parts nutrient broth |
|---------|--------------------------------|-----------------------------|--------------------------------------|-------------------------------------|--------------------------------------|----------------------|---------------------------------------------|-------------------------------|-----------------------------------------------------------------------|
|         | Triethanol-amine (Percent Wt.) | Caprylic Acid (Percent Wt.) | Copolymer <sup>1</sup> (Percent Wt.) | Parachloro-metacresol (Percent Wt.) | Parachloro-metaxylenol (Percent Wt.) | Phenol (Percent Wt.) | Orthobenzyl-parachloro-phenol (Percent Wt.) | Distilled Water (Percent Wt.) |                                                                       |
| 1       | 20                             | 3                           | 7                                    |                                     |                                      |                      |                                             |                               | 70                                                                    |
| 2       | 20                             | 3                           | 7                                    | 1                                   |                                      |                      |                                             |                               | Fail.                                                                 |
| 3       | 20                             | 3                           | 7                                    |                                     | 1                                    |                      |                                             |                               | Pass, no bacterial growth.                                            |
| 4       | 20                             | 3                           | 7                                    |                                     |                                      | 1                    |                                             |                               | Fail.                                                                 |
| 5       | 20                             | 3                           | 7                                    |                                     |                                      |                      | 1                                           | 69                            | Do.                                                                   |
|         |                                |                             |                                      |                                     |                                      |                      |                                             | 69                            | Do.                                                                   |

<sup>1</sup> Copolymer prepared from ethylene oxide and propylene oxide.

From the foregoing data of Tables I through IV, it will be apparent that the novel aqueous lubricant compositions of the present invention comprising a water-soluble alkanolamine, a saturated organic acid having from about 6 to about 9 carbon atoms per molecule, a water-soluble polyoxyalkylene glycol and a germicide, such as a halogenated cresol, exhibit outstanding properties from a standpoint of corrosion resistance, hard water stability, machining efficiency and efficacy in inhibiting bacterial growth. It will also be noted that the germicidal agents of the lubricant compositions of the present invention are effectively stabilized by the amine salt, i.e., the amine salt tends to solubilize the germicidal agent and thereby avoids precipitation of the latter, which would otherwise interfere with lubricating and machining efficiency. More specifically, with respect to the efficacy of the halogenated cresols in effectively inhibiting bacterial growth, it will be noted from Table IV that other closely related compounds, such as parachloro-meta-xylene, phenol or ortho-benzyl-para-chlorophenol, were unsatisfactory as indicated by excessive growth in the above-described biocide screening test.

While preferred embodiments of the compositions of the present invention and the method for their preparation have been described for purposes of illustration, it will be understood that various modifications and adaptations thereof, which will be obvious to those skilled in the art, may be made without departing from the spirit of the invention.

I claim:

1. A lubricant composition containing a major proportion of water, from about 5 to about 40 percent, by weight, of a water-soluble alkanolamine, from about 0.1 to about 9 percent, by weight, of a saturated organic acid having from about 6 to about 9 carbon atoms per molecule, selected from the group consisting of straight-chain organic acids and branched-chain organic acids, and from about 0.5 to about 20 percent, by weight, of a water-soluble polyoxyalkylene glycol.

35 and a halogenated cresol in an amount from about 0.05 to about 5 percent, by weight.

5. The lubricant composition of claim 4 wherein said alkanolamine is present in an amount from about 20 to about 35 percent, by weight; said organic acid is present in an amount from about 1 to about 4 percent, by weight; said polyoxyalkylene glycol is present in an amount from about 0.5 to about 5 percent, by weight; and said halogenated cresol is present in an amount from about 0.5 to about 3 percent, by weight.

6. The lubricant composition of claim 4 wherein said halogenated cresol is a chlorinated cresol.

7. The lubricant composition of claim 4 wherein said halogenated cresol is para-chloro-meta-cresol.

8. The lubricant composition of claim 4 containing as an additional component from about 0.1 to about 10 percent, by weight, of an alkali metal nitrite.

9. The lubricant composition of claim 4 containing as an additional component from about 0.1 to about 6 percent, by weight, of sodium mercapto-benzothiazole.

10. The lubricant composition of claim 4 containing as an additional component from about 0.1 to about 5 percent, by weight, of boric acid.

#### References Cited

#### UNITED STATES PATENTS

|           |        |                    |             |
|-----------|--------|--------------------|-------------|
| 2,605,206 | 7/1952 | Rowzet             | 167—38.7 XR |
| 2,625,509 | 1/1953 | Laug               | 252—34.7    |
| 2,825,693 | 3/1958 | Beaubien et al.    | 252—49.3    |
| 2,951,041 | 8/1960 | Saunders           | 252—34.7    |
| 3,201,349 | 8/1965 | Quanstrom          | 252—49.5 XR |
| 3,202,607 | 8/1965 | Koch               | 252—49.5    |
| 3,244,630 | 4/1966 | Sheikh             | 252—49.5    |
| 3,311,557 | 3/1967 | Schiermeier et al. | 252—49.5 XR |

DANIEL E. WYMAN, Primary Examiner.

C. F. DEES, Assistant Examiner.